

# UNITED STATES PATENT OFFICE.

DAVID E. REID, OF ROCHESTER, NEW YORK, ASSIGNOR TO EASTMAN KODAK CO., OF ROCHESTER, NEW YORK, A CORPORATION OF NEW YORK.

## MANUFACTURE OF ACETYL-CELLULOSE SOLUTIONS.

1,095,999.

Specification of Letters Patent.

Patented May 5, 1914.

No Drawing.

Application filed July 6, 1909. Serial No. 505,978.

*To all whom it may concern:*

Be it known that I, DAVID E. REID, of Rochester, in the county of Monroe and State of New York, have invented certain new and useful Improvements in the Manufacture of Acetyl-Cellulose Solutions; and I do hereby declare the following to be a full, clear, and exact description of the same.

My invention relates to the manufacture of relatively thin transparent sheets of acetyl cellulose of varying thickness suitable for supports for photographic film and for other purposes for which transparent flexible sheets are desirable. The most desirable manner of forming sheets of this character is by flowing a thick solution of the material upon a support having a polished surface and allowing the solvent to volatilize or evaporate, but difficulties are liable to arise by reason of the too rapid volatilization of the solvent employed and it is, therefore, the object of my invention to incorporate with the solvent a material which is not a solvent of acetyl cellulose but will, in a measure, retard the evaporation of the solvent during the formation of the sheet, and is necessarily of such nature that it will not have an appreciably deleterious effect upon the product when used for its intended purpose and will not affect or become affected by the substances or materials with which it is brought in contact during its manufacture or during its subsequent manipulation or future storage. If the solvent of the cellulose evaporates too rapidly, it is liable to form pits, lines in the surface of the sheet, or coagulate in hardened masses and form an uneven coating which will render the sheets unsuitable for such purposes, as, for instance, a support for photographic film. When these sheets are used as supports for photographic films, it is desirable and necessary that the retarding material used with the solvent have certain characteristics, as for instance: First: It must be of such a nature that it will not injuriously affect or interfere with the application of the sensitized coating. Second: It must have a relatively high boiling point, as compared with that of the solvent, in order that the sheet will cure out slowly and evenly. Third: It must be of such a nature that no chemical reaction will take place between it and the solvent or the cellulose. Fourth: It shall

have no effect upon the solvent or the cellulose to render it turbid or affect the transparency of the product. Fifth: It must have no chemical reaction with or on the ordinary metals. Sixth: It must not of itself be inflammable and must not increase the inflammability of acetyl cellulose, and seventh: It must not be oleaginous in character, as otherwise the surface of the sheet would be rendered objectionable for further treatment or the application of other materials. After considerable experimentation and research, I have discovered a material having these characteristics in pentachlorethane, one of the chlorin derivatives of ethane, having the formula  $C_2HCl_5$ , and a boiling point of 150° C.

In carrying out my invention I first dissolve the acetyl cellulose in a suitable solvent having a low boiling point, such as acetone or chloroform, in the proportion of about one part of cellulose to four of acetone or the other solvent, and to this add an amount of pentachlorethane equal to 50 to 100 per cent. of the weight of cellulose, and thoroughly incorporate the same by agitation. This thick viscous solution is then filtered and is coated in a thin coating upon a suitable support, and after drying or setting by the volatilization of the solvent it is stripped or removed for use. The action of the pentachlorethane retards the volatilization of the acetone or solvent to such an extent that the sheet is transparent, of uniform thickness, is free from pits or lines and irregularities, and its surface is smooth and of such nature that the sheets may be used for any purpose.

It will be noted that pentachlorethane having a high boiling point, a proportion of the same remains in the completed product from which the low boiling point solvent, as acetone, is eliminated by volatilization, and that the thin sheets formed as described are flexible, transparent, not readily inflammable, and are desirable as supports for a sensitized coating for photographic purposes, neither the coating nor the sheet being affected by the materials employed.

I claim as my invention:

1. A flowing solution of acetyl cellulose in a solvent having a low boiling point and containing a transparent liquid which is a non-solvent of cellulose, possessing a rela-

tively high boiling point, which is non-oleaginous in character and does not enter into chemical combination with the cellulose or the solvent employed, is not of itself inflammable and does not increase the inflammability of acetyl cellulose.

2. The flowing solution of acetyl cellulose in acetone containing pentachlorethane in an amount equal to fifty to one hundred 10 per cent. of the weight of the cellulose.

3. As a new composition of matter a solution of cellulose esters in pentachlorethane and organic solvents.

4. As a new composition of matter a solution of acetylcellulose in pentachlorethane and organic solvents.

5. As a new composition of matter a so-

lution of cellulose esters in pentachlorethane and acetone.

6. As a new composition of matter a so- 20 lution of acetylcellulose in pentachlorethane and acetone.

7. A composition of matter comprising acetyl cellulose containing pentachlorethane.

8. As a new composition of matter, a cel- 25 lulose ester containing pentachlorethane.

9. As an article of manufacture, a sheet of deposited or flowed acetyl cellulose containing pentachlorethane.

DAVID E. REID.

Witnesses:

GEO. EASTMAN.

ALICE K. WHITNEY.